

No. 836,520.

PATENTED NOV. 20, 1906.

A. MASSOTT, JR.

MANUFACTURE OF STEEL FROM ORDINARY IRON.

APPLICATION FILED JAN. 23, 1906.

Fig. 1. A--B.



Fig. 2. C--D.



Witnesses

J. M. Gowler, Jr.  
Rich. J. Hutchins

Inventor

Adam Massott, Jr.,  
By Mason, Fenwick, Lawrence  
F. W. S.

# UNITED STATES PATENT OFFICE.

ADAM MASSOTT, JR., OF MUTTERSTADT, GERMANY, ASSIGNOR TO FRITZ ANDRÉ, OF HAARDT, NEAR NEUSTADT A/H., GERMANY.

## MANUFACTURE OF STEEL FROM ORDINARY IRON.

No. 836,520.

Specification of Letters Patent.

Patented Nov. 20, 1906.

Application filed January 23, 1906. Serial No. 297,530.

*To all whom it may concern:*

Be it known that I, ADAM MASSOTT, Jr., merchant, a subject of the King of Bavaria, and a resident of Mutterstadt, in the Palatinate, Germany, have invented new and useful Improvements in the Manufacture of Steel from Ordinary Iron, of which the following is a specification.

My invention relates to a new process for preparing from ordinary iron steel the appearance and properties of which are equal to those of the best crucible cast-steel hitherto known.

The process is carried out in the way usual in cementing methods, the following mixture being used: three hundred grams yellow ferrocyanid of potassium, two hundred grams size prepared from leather parings, two hundred grams charcoal powder, one hundred and eighty grams colophony, twenty grams soda, forty grams finely-screened earth, twenty-five grams nitrate of potash, and thirty-five grams graphite. The iron masses to be converted are well packed in this powder and heated until bright red. The heat is maintained until the conversion has completely taken place. For bar-iron of ordinary dimensions this process requires about five hours. If it be desired to have only a partial conversion—that is to say, so that there should remain an inner iron core—the time will be correspondingly shortened. About one kilogram of the mixture is required for three and one-half kilograms of metal.

In carrying out the process it is essential that the muffle-furnace in which the iron to be converted is placed should be properly closed, so as to prevent the escape of the gases generated.

A furnace for carrying out the process is illustrated by way of example in the accompanying drawings.

Figure 1 is a longitudinal section on line A B of Fig. 2. Fig. 2 is a cross-section on line C D of Fig. 1.

a is a muffle made up of separate sections. This muffle in which iron bars or iron articles are placed in the powder described is covered by plates b in such manner as to produce round the muffle a chamber c, into which the combustion-gases from the grating f pass

through the slots g. From the chamber c the gases pass into the collector d, whence they escape into the chimney e. It will be seen that in this way on the one hand the 55 retorts are properly closed, and on the other hand, a good and uniform cooling of the same is attained.

Having now particularly described and ascertained the nature of my said invention 60 and in what manner the same is to be performed, I declare that what I claim is—

1. A method of manufacturing steel from ordinary iron and inferior sorts of steel, consisting in heating the metal in a furnace to 65 white heat, in contact with a material composed of ferrocyanid of potassium, leather size, carbon powder, colophony, finely-screened earth and soda with simultaneous addition of nitrate of potash and graphite, 70 substantially as described.

2. A method of manufacturing steel from ordinary iron and inferior sorts of steel, consisting in heating the metal in an air-tight 75 retort to white heat, and surrounding the metal with a material composed of ferrocyanid of potassium, leather size, carbon powder, colophony, finely-screened earth, graphite, potassium nitrate and soda.

3. The method of manufacturing steel 80 from ordinary iron and inferior grades of steel, consisting in heating the metal in a furnace to a white heat, in contact with a material composed of three hundred parts by weight of ferrocyanid of potassium, two 85 hundred parts by weight of size made from leather parings, two hundred parts by weight of powdered charcoal, one hundred and eighty parts by weight of colophony, twenty parts by weight of soda, forty parts by weight 90 of finely-screened earth, twenty-five parts by weight of potassium nitrate, and thirty-five parts by weight of graphite.

4. The method of manufacturing steel 95 from ordinary iron, and inferior grades of steel, consisting in heating the metal in an air-tight retort to a white heat, and surrounding the metal with a material composed of three hundred parts by weight of ferrocyanid of potassium, two hundred 100 parts by weight of size made from leather parings, two hundred parts by weight pow-

dered charcoal, one hundred and eighty parts by weight colophony, twenty parts by weight of soda, forty parts by weight of finely-screened earth, and twenty-five parts by weight of potassium nitrate, and thirty-five parts by weight of graphite.

In testimony that I claim the foregoing as

my invention I have signed my name, in presence of two witnesses, this 10th day of January, 1906.

ADAM MASSOTT, JUN.

Witnesses:

N. C. SCHLEMMER,  
Jos. H. LEUTE.